

Oct. 2, 1928.

1,686,353

W. M. TOWNE

PROCESS FOR WORKING ZINC

Filed July 27, 1925



Inventor

Walter M. Towne

By his Attorneys.

Fraser, Myers & Manley.

Patented Oct. 2, 1928.

## UNITED STATES PATENT OFFICE.

WALTER MARCUS TOWNE, OF NEW YORK, N. Y., ASSIGNOR, BY MESNE ASSIGNMENTS, TO E. W. BLISS COMPANY, OF BROOKLYN, NEW YORK, A CORPORATION OF DELAWARE.

## PROCESS FOR WORKING ZINC.

Application filed July 27, 1925. Serial No. 46,482.

This invention relates to the production of tubular zinc articles, especially in the form of cups or containers, by extrusion.

The present invention follows the method 5 claimed in my Patent No. 1,492,230, granted April 29, 1924, and constitutes a specific improvement thereon.

According to the process of that patent a blank of zinc, preferably soft zinc practically 10 free from grain formation and preferably zinc having a lead content not exceeding 0.6 per cent and a cadmium content not exceeding 0.5 per cent, is subjected to pressure between male and female dies and extruded through 15 the contracted annular space surrounding the male die in the direction opposite to the movement of the male die, and while at a temperature approximating 150° C. The present invention is based upon a later discovery and involves 20 essentially the extrusion at a considerably higher temperature approximating 260 to 300° C., whereby certain practical advantages are attained as compared with the process specifically set forth in my said prior patent, as will be explained.

In practising the process of the present invention I may use the same dies and tools as illustrated in my said Patent No. 1,492,230 and follow generally the same procedure with 30 respect to the selection of the zinc and the preparation of the zinc preparatory to the extrusion process. For these conditions it is sufficient to make reference to said patent, it being unnecessary here to repeat the detailed 35 discussion and directions therein contained.

The only difference made according to my present invention is in the temperature at which the extrusion is performed. This, instead of being "a temperature approximating 40 as closely as possible to 150° C.", as stated in my said patent, is a temperature materially above 150° C. and preferably approximating 260 to 300° C.

For the better understanding of my present 45 improvement I refer to the accompanying drawing, the single figure of which is a diagram showing the plasticity curve for zinc extrusion, that is to say, the pressures required at various temperatures for extruding zinc 50 battery cups as shown in said Patent No. 1,492,230 having an external diameter of 1.25 inch and side walls .014 inch thick. In this curve it will be noted that the point *a* is the one corresponding to the temperature of 150°

C. stated as preferable in my aforesaid patent. Below this temperature the pressure required for extrusion builds up with great rapidity and soon becomes so great as to be rapidly destructive to the die surfaces, thus causing a wasteful abrasion of the dies and 60 also requiring a high expenditure of power to operate the extrusion press. The point *b* indicates the temperature of 260 to 300° C., at which I preferably perform the extrusion according to the present invention. This elevation of temperature is accompanied by a diminution in pressure owing to the greater plasticity of the zinc at this higher temperature. Working at this temperature accomplishes an important economy in power, and 65 also a very serious advantage in the greater endurance of the dies. By reason of the more free flow of the metal there is apparently and probably some improvement in the quality of 70 the extruded cup.

I have even successfully worked at temperatures somewhat higher than 260 to 300° C., and even as high as 340 to 350° C., but these higher temperatures have no sufficient advantage in facilitating the operation, and 75 are subject to the disadvantage that they approach too closely to that at which the temper of the dies, or at least that of the male die or punch, is liable to be affected. As the dies for such work are quite expensive, it is 80 of great practical importance to give them the longest possible life, and any softening of the working faces of the dies due to the drawing of their temper causes their rapid deterioration. To avoid this, the temperature of the zinc while being worked should 85 not be carried so high as to cause this destructive effect upon the dies.

My present invention very materially increases the economy of production of zinc 90 battery cups and other similar zinc products by extrusion according to the process claimed in my said patent. This economy is due to more rapid operation, giving a higher output; to reduced cost for power; and to 100 prolonged life of the dies owing to their operating on the zinc in a condition which imposes less strain on the working faces of the dies.

At the time when I applied for my said 105 patent I stated that "at higher temperatures (than 150° C.) there is a decrease in its ductility" (referring to the zinc); and at that

- time such was my belief as the result of the experiments and tests I had theretofore made. My more recent experiments have led to the discovery that the ductility (or more correctly the plasticity) of the zinc increases as the temperature of extrusion is raised until a point is reached which approaches too closely to the melting temperature of the zinc, at which extrusion ceases to be possible.
- 10 The discovery of this fact has resulted from numerous experiments accompanied by many failures. During this time I had no means of ascertaining or determining the true ductility curve of zinc under extrusion conditions: this curve I have more recently been able to determine and plot as the result of said experiments and as the basis of the discovery underlying my present invention.

It is understood that while the present invention comes within the invention of my said prior patent, it excludes the specific temperature approximating 150° C. therein set forth.

What I claim is:

- 25 1. The process of working zinc which consists in subjecting a blank to pressure between male and female dies and extruding it through a contracted annular space surrounding the male die in a direction opposite to the movement of the male die and while at

a temperature approximating 260 to 300° C., in substantially the manner set forth.

2. The process of working zinc which consists in subjecting a blank to pressure between male and female dies and extruding it through a contracted annular space surrounding the male die in a direction opposite to the movement of the male die and while at a temperature exceeding 260° C. and not materially exceeding 300° C.

3. The process of working zinc which consists in subjecting a blank to pressure between male and female dies and extruding it through a contracted annular space surrounding the male die in a direction opposite to the movement of the male die and while at a temperature approximating 300° C., substantially as set forth.

4. The process of working zinc which consists in subjecting a blank to pressure between male and female dies and extruding it through a contracted annular space surrounding the male die in a direction opposite to the movement of the male die and while at a temperature materially exceeding 150° C. and not materially exceeding 300° C.

In witness whereof, I have hereunto signed my name.

WALTER MARCUS TOWNE.